

# UNITED STATES PATENT OFFICE.

CHARLES J. NETHERCOTT, OF SALT LAKE CITY, UTAH.

## COMPOSITION FOR WATERPROOFING LEATHER, CANVAS, AND OTHER CLOTH.

1,359,826.

Specification of Letters Patent. Patented Nov. 23, 1920.

No Drawing.

Application filed May 13, 1919. Serial No. 296,948.

To all whom it may concern:

Be it known that I, CHARLES J. NETHERCOTT, a citizen of the United States, residing at Salt Lake City, in the county of Salt Lake and State of Utah, have invented certain new and useful Improvements in Composition for Waterproofing Leather, Canvas, and other Cloth, of which the following is a specification.

10 The object of my invention is to provide a composition of matter which may be used to treat leather upholstering such as the top and seats of automobiles to render them waterproof, and also to treat the tops and seats when made of canvas or other cloth with the same composition of matter to render them waterproof and leave the leather and cloth after treatment soft and pliable. Also to treat canvas bags and sacks so that 15 the material held in such bags and sacks will not become useless on account of water entering the sacks, and at the same time to retain all of the material carried in said sacks or bags, such as Portland cement, 20 plaster of Paris and many other dust like preparations, and these objects I accomplish by filling the pores and interstices with a pliable waterproof matter which adheres to the fabrics and which will not be sticky 25 to 30 nor yet brittle enough to crack when the treated material is bent or creased.

My composition consists of the following ingredients, combined in the proportions stated, viz:

35 Five quarts of good quality varnish for outside use.

Three quarts of japan sizing, which is a composition of 1 part coach japan with one part japan gold sizing. The coach japan is made of manganese oxid, linseed oil and naphtha. The japan gold sizing is made of fossil gums, rosin, linseed oil, naphtha and manganese oxid.

Eight quarts of paint.

45 25 ounces of bees wax.

25 ounces of glycerin.

10 ounces of eucalyptus oil.

6 teaspoonfuls of sweet oil.

Two gallons of a thinner such as turpen-

50 tine or gasoline.

These ingredients are to be thoroughly mingled by heat and agitation.

To properly prepare and mix the ingredients, I take two quarts of the lightest colored durable varnish. Three quarts of

"spar" varnish, 1½ quarts pale coach japan, which is a composition of manganese oxid, linseed oil and naphtha, 1½ quarts of japan gold sizing, which is a combination of fossil gums, rosin, linseed oil, naphtha and 60 manganese oxid, 25 ounces of glycerin, 10 ounces of eucalyptus oil, six teaspoonfuls of sweet oil, and shave into thin strips or small particles 25 ounces of bees wax which is added to the above liquids, then heat the 65 wax and all of the other ingredients by placing the vessel in which they are mixed in hot or boiling water, but not over a direct fire, until the wax is melted. When this mixture is cooled add the thinner, of two 70 gallons of turpentine or gasoline, and thoroughly mix. If the compound is for use on leather or other fabric where a black or dark color is desired I add to the first mixture before heating it 1½ quarts of black 75 enamel paint, six quarts of black asphalt and 5 pounds of jet black coach paint. If the compound is for use on canvas or other cloth of light colors or where light colors such as white, aluminum, blue or yellow are 80 desired, I do not use the black enamel, asphalt or black coach paint but use instead, white enamel 1½ quarts, and five pounds of painter's flake white paint which is carbonate of lead ground in oil, with 1½ quarts 85 of any desired color paint or pigment.

By using my composition I am able to treat leather upholstering such as tops on automobiles to restore the finish and make the leather water proof and pliable by applying the compound to the leather upholstering and allowing it to dry. I am also able to treat the canvas or other cloth upholstering by covering and saturating the cloth, whether old or new, with a water- 95 proofing compound which will render the cloth pliable and moisture resistant, and give it any desired color by mixing the ingredients as above set out.

In treating canvas or other cloth I apply 100 the mingled ingredients with a paint brush, giving it one coat, then after said coat has dried, which will take about six hours, I apply another coat and allow it to dry, without rubbing. I advise the thorough agitation of the compound before use in order to avoid any tendency of the solids to settle in the bottom of the container, however the glycerin content will preserve the solids in a fluid and plastic condition.

Having thus described my invention I desire to secure by Letters Patent and claim:—

1. A waterproofing composition consisting of five quarts of good quality varnish; three quarts of japan sizing; eight quarts of black paint; twenty-five ounces of bees wax; twenty-five ounces of glycerin; ten ounces of eucalyptus oil; six teaspoonfuls of sweet oil; and two gallons of turpentine, substantially as described.

2. A waterproofing composition consisting of five quarts of good quality varnish; three quarts of japan sizing; eight quarts of paint; twenty-five ounces of bees wax; twenty-five ounces of glycerin; ten ounces

of eucalyptus oil; six teaspoonfuls of sweet oil; and two gallons of turpentine, substantially as described.

3. A waterproofing composition consisting of two quarts of light colored durable varnish; three quarts of "spar" varnish;  $1\frac{1}{2}$  quarts of coach japan;  $1\frac{1}{2}$  quarts of japan gold size;  $1\frac{1}{2}$  quarts of enamel paint; five pounds of coach paint;  $1\frac{1}{2}$  pounds of pigment any desired color; twenty-five ounces of melted bees wax; twenty-five ounces of glycerin; ten ounces of eucalyptus oil, and two gallons of turpentine.

In testimony whereof I have affixed my signature.

CHARLES J. NETHERCOTT.